

## UNITED STATES PATENT OFFICE

2,058,344

LUBRICANT AND METHOD OF MAKING  
SAME

Robert C. Moran, Wenonah, and William L. Evers and Everett W. Fuller, Woodbury, N. J., assignors to Socony-Vacuum Oil Company, Incorporated, New York, N. Y., a corporation of New York

No Drawing. Application November 16, 1935,  
Serial No. 50,238

## 4 Claims. (Cl. 87—9)

The design of automotive engines is at present tending toward the use of higher compression and higher rotative speeds and is encountering higher crankcase temperatures and higher bearing pressures. This is resulting in a departure from the use of bearing metals of the usual types such as babbitt. The bearing metals coming into the general use are of different natures, but as a general thing although they are harder, they 5 are more susceptible to destructive agencies of a corrosive nature. Typical of these newer bearing metals are those composed of cadmium-silver alloys, cadmium-nickel alloys, and copper lead alloys. One widely used type of bearing of 10 the newer kind is composed of a cadmium-silver alloy supported upon a steel back.

Concurrent with changes in engine design have been marked advances in methods of refining lubricant oils for automotive use, due to the sharp demand for oils having a low rate of 15 change of viscosity with temperature; that is oils of a high viscosity index (V. I.). This demand for such oils has been met by refining lubricants intended for motor oils with certain solvent extraction processes. In these processes 20 advantage is taken of the fact that numerous reagents, such as for example dichlorodioethyl-ether, cresylic acid, phenol, chloraniline, chlorophenol, phenetidine, benzyl alcohol, nitrobenzene, benzonitrile, furfural, aniline, benzyl acetate, liquid sulphur dioxide, a mixture of liquid sulphur dioxide or aniline with benzol, and the like, have selective solvent power for hydrocarbons of various types. These solvent refining processes are operated in a manner which 25 concentrates in the desired lubricating fractionation, those compounds of a "paraffinic" nature which have a low susceptibility to change of viscosity with change in temperature or in other words, a high viscosity index. In doing 30 this, they reject from the desired lubricant those compounds of "naphthenic" nature which have a low viscosity index. These processes have enabled the supply of an oil of highly desirable 35 general characteristics definitely far superior to any oil previously produced from mixed base or asphaltic crudes and superior to a like, although lesser, degree over oils previously produced from paraffin base crudes. It has been found that 40 45 50 motor oils produced by the solvent refining process referred to above are definitely corrosive to the newer bearing metals under normal conditions of automotive use, and in extreme cases their corrosive properties have been so great as 55 to result in bearing failure after only a few

thousand miles of normal driving. It is further known that the same reaction, viz., corrosion of alloy bearing metals such as cadmium-silver, also occurs in good paraffinic base oils which have not been subjected to solvent refining. The degree of corrosiveness apparently rises with the viscosity index, since with oils of higher viscosity index, the tendency to corrosion of the kind referred to above is more pronounced. Speaking in general terms, corrosion of this nature is 5 encountered to a recognizable degree in oils having a V. I. of 75 or higher, becoming important in amount in oils having a V. I. of 80 to 85 or higher, and very serious in nature in oils of 100 V. I. or higher.

It is an important object of this invention to provide means for satisfactorily inhibiting or preventing this corrosion from taking place to a serious degree. It is an object of this invention to alter or modify a highly refined motor oil, 20 normally corrosive, by use of an additive ingredient capable of substantially inhibiting this corrosion. It is an object to provide a substantially non-corrosive motor oil of high V. I. An object of this invention is to provide an additive reagent or ingredient capable of inhibiting the corrosive properties of these oils. The production of solvent refined oils of low corrosive properties under conditions of automotive use is a major object of this invention, as well as the 25 method of production of such oils which couple high viscosity index with low tendency to corrosion.

This invention is based on the discovery that the addition to the oil of small amounts of a tricresylphosphite ( $(CH_3C_6H_4O)_3P$ ), accomplishes 30 the above object. It is found that when corrosion of the type referred to above occurs, especially if it occurs in the presence of a motor oil which has been produced by a process of solvent refining, in which type of oil the corrosive properties appear to be more marked, that the oil can be rendered substantially non-corrosive under 35 conditions much more strenuous than normal automotive use by the addition of controlled amounts of this compound, viz., a tricresylphosphite. The tricresylphosphites are isomeric organic compounds having the following graphic formula:



This compound may be prepared by the reaction of ortho-cresol or meta-cresol or para-cresol or 55

mixtures thereof and phosphorous trichloride, in the proportions of three molecular amounts of the cresol or mixed cresols to one molecular amount of phosphorous trichloride. The reaction mixture is heated until the evolution of hydrogen chloride ceases. The resulting product, a tricresylphosphite, may be purified if desired by a process of fractional distillation. For the present objects, it may be used either as produced or 10 in the fractionated form. A satisfactory reaction product may be made by heating the reaction mixture after the cessation of the evolution of HCl gas to a temperature of 200° C. under a pressure of 2 mm. mercury. The product so made 15 is designated hereinafter as topped. The following data demonstrate the effectiveness of this novel corrosion inhibitor. In these tests a motor oil of S. A. E. 20 rating, having a Saybolt viscosity of 56.6' at 210° F., a flash point of 425° F. and a 20 V. I. of 117 was used, this oil being an oil which had been subjected to a high degree of solvent refining. Actual motor operation tests are set forth in Table I below. In these tests, a motor oil blank and motor oil blends containing different 25 proportions of the novel corrosion inhibiting ingredient of this invention were subjected to test in a modified Delco knock test engine, equipped with bearings of cadmium-silver alloy on a steel back. The alloy is about 2.5% silver, a few hundredths of a per cent of copper and the balance of cadmium. The motor was equipped with crankcase oil heaters to maintain oil temperatures (330° F.) at least equal to those encountered 30 under extreme conditions of automotive use. On 35 each test, the test engine was operated for 40 hours, at a rotative speed the equivalent of an automobile road speed of 60 miles per hour. In rough terms each test is the equivalent of exposure of the oil to use in an automobile for 2400 40 miles of continuous driving at 60 miles per hour, a condition far more rigorous than any encountered in normal use. The bearings in the engine were new for each test and were carefully weighed before and after to determine loss of weight. 45 The neutralization number (N. N.) of the used oil was measured and is recorded as being indicative of the corrosive nature of the oil. The inhibitor used was the mixed isomeric tricresylphosphite described above.

50

Table I

| 55                    | Time          | Results of Delco test engine on S. A. E. 20 oil containing 3% tricresylphosphite |                                      |                        |
|-----------------------|---------------|----------------------------------------------------------------------------------|--------------------------------------|------------------------|
|                       |               | N. N. of oil                                                                     | Grams loss of cadmium-silver bearing | Bearing wear in inches |
| 60                    | 20 hours..... | 0.25                                                                             | 0.2173                               | .0002"                 |
|                       | 40 hours..... | 1.70                                                                             | 0.3465 (total)                       | .0002" (total)         |
| S. A. E. 20 oil alone |               |                                                                                  |                                      |                        |
| 65                    | 20 hours..... | 5.12                                                                             | 4.920                                | .004"                  |

An indicative test of considerable merit may be made in the laboratory by suspending a portion of a cadmium-silver alloy bearing in a bath of the oil 70 under test in a glass container, maintaining the oil at about 350° F., and passing air through the oil in contact with the bearing metal. Convenient conditions are: 30 gm. oil, 2,000 ml. air per 75 hour, 22 hours. The following table shows re-

sults of a series of such tests in which oils containing different proportions of tricresylphosphite, and an oil blank were tested, giving the loss in weight of the bearing metal, and the neutralization number of the used oil. The oil used 5 was the same as in Table I.

Table II

|                                                | Cadmium-silver bearing weight change in milligrams | N. N. of used oil | 10 |
|------------------------------------------------|----------------------------------------------------|-------------------|----|
| Oil blank (S. E. A. 20).....                   | -38.3                                              | 2.60              | 15 |
| Oil with 0.10% triorthocresyl-phosphite.....   | +0.2                                               | 0.42              |    |
| Oil with 0.25% triorthocresyl-phosphite.....   | -0.5                                               | 0.64              |    |
| Oil blank (S. A. E. 20).....                   | -68.7                                              | 2.30              |    |
| Oil with 0.10% mixed tricresyl-phosphites..... | -1.8                                               | 0.40              |    |

From these tests, it is evident that the use of this 20 novel corrosion inhibitor, viz., tricresylphosphite, in amounts as small as 0.10% prevented corrosion to a substantially complete degree under conditions much more rigorous than any likely to be met in practice.

From the combined evidence of the above exemplary data, it is evident that the novel corrosion inhibiting ingredients herein disclosed, namely tricresylphosphites are effective agents for the prevention of corrosion of automotive 30 parts, particularly the newer type alloy bearings, when introduced in proper amounts into an oil otherwise highly corrosive.

Visual examination of the bearings from engine tests such as those reported in Table I show 35 the effectiveness of tricresylphosphites in a very marked manner. The bearing subjected to the oil blank shows plainly the effect of corrosion, very little of the original surface remaining. The bearings subjected to the inhibited oils show little 40 or no visual evidence of corrosion. Similar visual evidence of the effectiveness of this inhibitor may be noted by inspection of the pieces of metal used in the tests in glass.

It is preferred to use this ingredient, a tricresylphosphite, in amounts ranging between 45 0.25% and 1.0% although for less severe services and in oils not highly corrosive, as low as 0.10% may be fully effective for the purpose intended.

These ingredients, tricresylphosphites, are 50 water clear oils freely miscible with hydrocarbons, and may be added in any proportion without darkening or deepening the color of the oil. When so added, they have no tendency to separate from the oil under conditions of storage or 55 use.

We claim:

1. A method of lubricating bearing surfaces in 60 internal combustion engines when subjected to conditions of operation which comprises maintaining between bearing surfaces, one of which is an alloy formed chiefly of a metal selected from the class consisting of cadmium and copper, a film of lubricating oil which initially produces an effective lubricating action but which would normally tend to corrode the aforesaid alloy, and maintaining the effectiveness of the lubricating oil by incorporating therein tricresylphosphite in a small but sufficient proportion substantially to retard the corrosion.

2. A method of lubricating bearing surfaces in 65 internal combustion engines when subjected to conditions of operation which comprises maintaining between bearing surfaces, one of which is an alloy formed chiefly of a metal selected from 70

the class consisting of cadmium and copper, a film of lubricating oil which initially produces an effective lubricating action but which would normally tend to corrode the aforesaid alloy, and maintaining the effectiveness of the lubricating oil by incorporating therein from 0.1% to 1.0% of tricresylphosphite sufficient substantially to retard the corrosion.

3. A method of lubricating bearing surfaces which comprises maintaining between bearing surfaces, one of which is an alloy selected from the class consisting of cadmium-silver, cadmium-nickel, and copper-lead alloys, a film of lubricating oil which initially produces an effective lubricating action but which would normally tend to corrode the aforesaid alloy, and maintaining the effectiveness of the lubricating oil by incorporating therein from 0.1% to 1.0% of tricresylphosphite sufficient substantially to retard the corrosion.

ing therein tricresylphosphite in a small but sufficient proportion substantially to retard the corrosion.

4. A method of lubricating bearing surfaces which comprises maintaining between the bearing surfaces, one of which contains a characterizing proportion of cadmium, silver, nickel, copper or lead, a film of lubricating oil which initially produces an effective lubricating action but which would normally tend to corrode the aforesaid surface, and maintaining the effectiveness of the lubricating oil by incorporating therein tricresylphosphite in a small but sufficient proportion to substantially retard the corrosion.

ROBERT C. MORAN.

WILLIAM L. EVERS.

EVERETT W. FULLER.

5

10

15